

## UNITED STATES PATENT OFFICE.

BO MICHAEL STURE KALLING AND SVEN DAGOBERT DANIELI, OF TROLLHATTAN, SWEDEN, ASSIGNORS TO AKTIEBOLAGET FERROLEGERINGAR, OF STOCKHOLM, SWEDEN, A LIMITED JOINT STOCK COMPANY.

PROCESS FOR THE MANUFACTURE OF METALS OR ALLOYS POOR IN CARBON AND SILICON.

No Drawing.

Application filed February 1, 1922. Serial No. 533,381.

*To all whom it may concern:*

Be it known that Bo MICHAEL STURE KALLING and Sven DAGOBERT DANIELI, engineers, subjects of the King of Sweden, residing at Trollhattan, in the Kingdom of Sweden, have invented new and useful Improvements in Processes for the Manufacture of Metals or Alloys Poor in Carbon and Silicon, of which the following is a specification.

This invention relates to the manufacture of metals or alloys having a low percentage of carbon and silicon, the principal object of the invention being to provide a process whereby such metals or alloys can readily be manufactured in an electric furnace without the passage of carbon into the charge during the process.

The present invention is based upon the fact that silicon has the property of being able to expel carbon from a metal or alloy. Consequently, an alloy having a high percentage of silicon necessarily has a low percentage of carbon. Therefore, in order to produce as a final product a metal or alloy poor in both carbon and silicon, it is necessary to start with an alloy rich in silicon, which alloy may be produced in any desired manner. It is preferable that this alloy contain at least 10 per cent of silicon, since, if a smaller percentage be present, the content of carbon will not have decreased sufficiently to be regarded as "low." If preferred, more or less pure silicon, for example, in the form of high per cent ferro-silicon, may be employed. This alloy, rich in silicon, is then melted, together with substances containing oxides of metals which are capable of oxidizing silicon, such, for instance, as the oxides of chrome, vanadium, manganese, tungsten, iron, nickel, and the like, and if necessary a suitable flux, such for instance as lime, magnesia, or the like, may be added to the molten mass.

If the process can be carried on under such conditions as to obviate the absorption of carbon by the charged raw material or by the products formed, the metal or alloy produced will obviously not contain, absolutely speaking, a larger quantity of carbon than that charged with the raw material, and is thus, poor in carbon and silicon, pro-

vided the oxidation of the silicon has been carried sufficiently far.

As a general rule, in order to get the oxidation of the silicon started, it is necessary that the heating should take place at such a high temperature that the electric furnace is the only suitable apparatus for the purpose. The furnace, however, must be so constructed that it works with a free electric arc, that is, so that its electrodes do not come into contact with the charge, as otherwise the carbon from the electrodes will be absorbed by the charge, and this is especially true in the treatment of substances which contain one or more of the oxides of chrome, vanadium, manganese, or tungsten.

It is, however, known that in such electric furnaces the energy supplied is badly utilized, and moreover, that the part or parts of the lining which are directly exposed to the radiation from the electric arc are rapidly consumed, both of which circumstances entail comparatively poor economic results. It is also known that the two drawbacks just mentioned in the electric furnace working with a free electric arc are considerably lessened in that type of electric furnace where the electric current, wholly or partially, must pass from one or more movable electrodes directly to the charge.

To be able to use an electric furnace of the latter type for the process in question is therefore a desideratum, the realization of which has hitherto been frustrated by the fact that the charge absorbs carbon from the electrode or electrodes. The inventors of the present invention have, however, discovered that an electric furnace of the type above referred to can be used for the above-mentioned process of manufacturing metals or alloys poor in carbon or silicon—without any carbon, practically speaking, passing into the charge—if the electric power is supplied under such a voltage that the effective ohmic voltage drop between the point of the electrode, or electrodes, which supply the electric current to the charge and the charge itself is not permitted to fall below 70 volts during the process.

The inventors have, moreover, ascertained

that the kind of system adopted—whether single-phase or polyphase alternating current, or direct current—does not affect the result.

5 In order that the reaction between the silicon of the charged alloy rich in silicon, on the one hand, and the oxides supplied for the oxidation of the silicon, on the other, may be carried sufficiently far, the oxides must be 10 present in a certain excess. The inventors have, however, ascertained that this excess can be lessened in proportion to the fineness of grain of the reagents and the thoroughness of the mixture and that the minimum 15 excess of oxidizing agents may be used when the mixture of the finely crushed materials is supplied to the furnace in the form of briquettes.

In the manufacture of the briquettes, any 20 binding mediums employed must, of course, be practically free from carbon. Water-glass, clay, cement, etc., have been found to be suitable binding media for this purpose. It is likewise advantageous that the bri- 25 quettes, before use, should have been heated to such a high temperature that all traces of moisture have been expelled, for which purpose the briquettes in general require to be heated to a temperature of over 500°.

30 The above stated process for the manufacture of metals and alloys poor in carbon and silicon has, after thorough experiments, been used by the inventors with success for the manufacture of chrome manganese, van- 35 dium, and tungsten, and for the manufacture of alloys of those substances with iron, nickel, or both.

In order further to make plain the invention, an example will be given of the manu- 40 facture of ferro-manganese poor in carbon and silicon in accordance with the above stated process.

A silico-manganese alloy containing, for example, 22 per cent of silicon, and less than 45 1 per cent of carbon, is ground to fine powder, and is thoroughly mixed with finely ground manganese ore, previously heated to redness and with ground, dead dolomite in suitable proportions. The mixture is bri- 50 quetted with a solution of water-glass as a binding medium, whereupon the briquettes are dried and baked.

An electric furnace with a single adjustable electrode, and with a lining which does 55 not contain carbon, is supplied with electric power in the form of a single-phase alternating current with such high voltage that the effective ohmic voltage drop between the point of the electrode, and the lining of the 60 furnace will have a minimum value of 70 volts. The electrode is brought sufficiently close to the furnace bottom to cause an electric arc to arise between the bottom and electrode. When the arc has been maintained 65 for a sufficient length of time to enable the

furnace lining to become warmed the furnace is charged with a suitable quantity of the briquettes manufactured in the manner described above, whereupon the smelting im- 70 mediately begins—provided that the load on the furnace, by the regulation of the adjustable electrode in the furnace, is main- 75 tained at a suitable amount. From the moment when the resistance of the charge itself is put in circuit, care must be taken that the effective voltage drop between the point of the electrode and the charge is maintained above 70 volts, for which purpose it may be necessary to raise the voltage supplied to the furnace. When the first charge of briquettes 80 has melted, the furnace is charged with a fresh quantity, and this procedure is continued until a suitable total quantity has been smelted, whereupon the content of the fur- 85 nace is tapped off, the furnace is charged with a fresh quantity of briquettes, and so forth. If the percentage of ore in the briquettes has been properly adjusted, the ferro- 90 manganese obtained will contain less than 1% of carbon and less than 2% of silicon. The slag simultaneously obtained will contain about 30% of Mn, and can suitably be used as raw material for the manufacture of silico-manganese. It will be understood, 95 of course, that the expression "process of manufacturing metals" used in the claims is intended to cover not only manufacturing of metals as such, but also alloys of metals.

Having thus described our invention we declare that what we claim is:

1. The process of manufacturing metals poor in carbon and silicon, which consists in producing an alloy rich in silicon, mixing with said alloy an agent capable of oxidizing silicon, heating the mixture in an electric furnace, and maintaining the effective ohmic voltage-drop between the points of the electrodes of the furnace and the charge above 70 volts.

2. The process of manufacturing metals poor in carbon and silicon, which consists in producing an alloy rich in silicon, mixing with said alloy a flux and an agent capable of oxidizing silicon, heating the mixture in an electric furnace, and maintaining the effective ohmic voltage-drop between the points of the electrodes of the furnace and the charge above 70 volts.

3. The process of manufacturing metals poor in carbon and silicon, which consists in producing an alloy containing at least 10 per cent of silicon, mixing with said alloy an agent capable of oxidizing silicon, heating the mixture in an electric furnace, and main- 120 taining the effective ohmic voltage-drop be- 125 tween the points of the electrodes of the fur- nace and the charge above 70 volts.

4. The process of manufacturing metals poor in carbon and silicon, which consists in producing an alloy rich in silicon, mixing 130

with said alloy an oxide of a metal capable of oxidizing silicon, heating the mixture in an electric furnace, and maintaining the effective ohmic voltage-drop between the 5 points of the electrodes of the furnace and the charge above 70 volts.

5. The process of manufacturing metals 10 poor in carbon and silicon, which consists in producing an alloy containing at least 10 per cent of silicon, mixing with said alloy chromium oxide, heating the mixture in an electric furnace, and maintaining the effective ohmic voltage-drop between the points of the electrodes of the furnace and the 15 charge above 70 volts.

6. The process of manufacturing metals 20 poor in carbon and silicon, which consists in producing an alloy rich in silicon, mixing with said alloy a flux and chromium oxide, heating the mixture in an electric furnace, and maintaining the effective ohmic voltage-drop between the points of the electrodes of the furnace and the charge above 25 70 volts.

7. The process of manufacturing metals 30 poor in carbon and silicon, which consists in producing an alloy rich in silicon, mixing with said alloy an excess of an agent capable of oxidizing silicon, heating the mixture in an electric furnace, and maintaining the effective ohmic voltage-drop between the points of the electrodes of the furnace and the charge above 35 75 70 volts.

8. The process of manufacturing metals 40 poor in carbon and silicon, which consists in producing an alloy rich in silicon, pulverizing said alloy and mixing therewith a pulverized agent capable of oxidizing silicon, heating the mixture in an electric furnace, and maintaining the effective ohmic voltage-drop between the points of the electrodes of the furnace and the charge above 45 80 70 volts.

9. The process of manufacturing metals 50 poor in carbon and silicon, which consists in producing an alloy rich in silicon, pulverizing said alloy and mixing therewith a pulverized agent capable of oxidizing silicon, binding said mixture together in the form of briquets, heating said briquets in an electric furnace, and maintaining the effective ohmic voltage-drop between the points of the electrodes of the furnace and the charge above 55 85 70 volts.

10. The process of manufacturing metals

poor in carbon and silicon, which consists in producing an alloy rich in silicon, pulverizing said alloy and mixing therewith a pulverized agent capable of oxidizing silicon, adding to said mixture a binding material 60 free from carbon, forming said mixture into briquets, heating said briquets in an electric furnace, and maintaining the effective ohmic voltage-drop between the points of the electrodes of the furnace and the charge above 65 70 75 70 volts.

11. The process of manufacturing metals 70 poor in carbon and silicon, which consists in producing an alloy rich in silicon, pulverizing said alloy and mixing therewith a pulverized agent capable of oxidizing silicon, adding to said mixture a solution of water-glass and forming the same into briquets, heating said briquets in an electric furnace, and maintaining the effective ohmic voltage-drop between the points of the electrodes of the furnace and the charge above 75 75 70 volts.

12. The process of manufacturing metals 80 poor in carbon and silicon, which consists in producing an alloy rich in silicon, pulverizing said alloy and mixing therewith a pulverized agent capable of oxidizing silicon, adding to said mixture a binding substance free from carbon, and forming said mixture into briquets, heating said briquets to a temperature of at least 500° C., charging the briquets into an electric furnace, and maintaining the effective ohmic voltage-drop between the points of the electrodes of the furnace and the charge above 85 80 75 70 volts.

13. The process of manufacturing ferro-chromium poor in carbon and silicon, which 90 consists in producing an alloy of chromium rich in silicon, mixing with said alloy an excess of chromium ore, heating said mixture in an electric furnace, and supplying current to the furnace at such a voltage that the effective ohmic voltage-drop between the points of the electrodes of the furnace and the charge is maintained above 95 70 volts.

In testimony whereof we have signed our names to this specification.

BO MICHAEL STURE KALLING.  
SVEN DAGOBERT DANIELI.

Witnesses:

AUG. HAGELIN,  
E. MIRON.